

July 29, 1947.

C. A. HOGAN

2,424,825

METHOD OF REPAIRING OPEN HEARTH FURNACE BANKS

Filed Jan. 16, 1945



INVENTOR.

BY *Charles A. Hogan,*  
*Charles O. Henry,*  
*his atty.*

## UNITED STATES PATENT OFFICE

2,424,825

METHOD OF REPAIRING OPEN HEARTH  
FURNACE BANKS

Charles A. Hogan, Chicago Heights, Ill.

Application January 16, 1945, Serial No. 573,071

3 Claims. (Cl. 25—155.5)

1

This invention relates to a method of repairing or patching the banks of open hearth furnace bottoms. The principal object of the present invention is to make repairs of furnace banks, which repairs are more efficient than the present day repairs, and to minimize the cost of such repairs.

It is well known to those skilled in the art to which this invention pertains, that the molten metal cuts or washes away furnace banks at the slag line; consequently, repairs must be made after each heat to restore the bank to normal usable condition.

One object of the invention is to provide a thin layer of slag over the refractory material which is used to fill in the cavities, which layer of slag fuses at a considerably lower temperature than the refractory materials, and trickles down through them causing a firmer bond between the materials and more effectively resisting the destructive action of the molten metal at the slag line on the bank.

With these and other advantages in view this invention consists in the novel method herein-after fully described and claimed.

The method of carrying out the invention is illustrated in the accompanying drawing in which the figure is a cross section of a conventional open hearth furnace showing a break in the bank and a repaired cavity.

Referring to said drawing, the reference character 1 designates an open hearth furnace of conventional construction, having a bed bottom 2, of refractory materials constructed in the customary manner with the bank 3, sloping toward the door openings, one of which is seen at 4.

A cavity caused by the action of the molten metal is seen at 5, and at 6 is shown a cavity which is being repaired in accordance with the present method. The cavity may extend around the entire bank and frequently does so.

After the heat has been drawn off, relatively inexpensive refractory material 7, such as dolomite, magnesite or the like is thrown through the door openings into the cavities in the bank, after which a thin layer of slag 8 is thrown upon the refractory material. Because of the low fusion point of the slag, it melts and trickles down through the refractories and effectively binds them together.

If a cavity is relatively shallow, it may be filled with the refractory material to the original bank surface, and the layer of slag is then spread over the filled in refractory material. If the cavity is relatively deep, it is preferred to only partially

2

fill it with refractory materials and add a layer of slag and then fuse this layer before fusing the next layer, and subsequently continue the same process until the cavity has been built up to the original bank surface. When the slag fuses, it trickles down into the refractory material.

Since the layer of slag is relatively thin, the heat does not have to penetrate so far as when the slag is mixed with the refractories, consequently the slag is fused quicker and trickles down into the refractories acting as a flux therefore, and making a solid bond between them.

Furthermore, inasmuch as the fusion point of slag is much lower than the refractory materials 15 the furnace can be operated at less damaging temperatures than heretofore. The furnace being charged, it is operated at full blast with no attention paid to temperature and since the slag is applied to the outside surface of the repair materials, the fusion point of the refractory materials is diluted, thus increasing the thickness of the surface crust that is formed over the cavity thereby providing a more efficient repair job.

In repairing banks of open hearth furnaces, 25 the refractory materials and the slag may be thrown into the cavities with a shovel or with any suitable apparatus. I have found that great efficiency is obtained by adding about 8 to 10 pounds of slag, evenly scattered, over each lineal foot.

From the above it is apparent that with my method, a bonded bank to a depth of two inches to four inches, more or less is possible according to the size of material used and length of time available before the iron is added, whereas the present day practice consists in fusing only a very thin crust of probably one quarter to one half inch at most.

Since the face of added repair material receives the brunt of flame heat, the outside section of the ordinary bank repair material fuses together closing all voids and crevices and prevents the heat from penetrating the necessary depth to fuse all or even very much of the added material; 40 because of this condition the ordinary material used in the repair of the bank does not give fullest efficiency because of the lack of slag to fuse it quickly.

In accordance with my method, cheaper repair materials may be used more efficiently and can replace the more expensive materials in many plants, thereby effecting great savings.

The use of dolomite or magnesite for making repairs requires some slag to fuse properly, but 45 with a covering of slag as is practiced with my

method those materials are fused to a much greater depth than heretofore.

In accordance with my method, where slag is added early, and a subsequent part of the charge is added after the furnace has become quite hot from melting the first charge of scrap, the hot and fused bank becomes chilled or "set" as it is termed, which in itself is very important, and manifestly without the slag facing the bank repair would not be nearly so well fused.

With the proper addition of slag to the surface a more efficient bank repair is attained, there is a saving in expensive repair materials, with no loss of time, and effectively preventing many break-outs of steel before heats are ready.

I claim as new and desire to secure by Letters Patent:

1. The method of restoring worn away portions of open hearth furnace banks to normal usable condition, which consists in filling in the cavities in the bank with discrete refractory material, and covering said refractory material with a relatively thin layer of slag directly after a heat, and subjecting the slag to the influence of sufficient heat to fuse the same and permit it to trickle into the refractory material, whereby to bond the refractory repair material together.

2. The herein-described method of restoring worn away portions of open hearth furnace banks to normal usable condition which consists in filling in the cavities in the bank with discrete refractory material, covering said refractory material with a layer of slag directly after a heat, fusing the slag and permitting it to trickle into the refractory material, whereby to bond the refractory repair material together.

3. The method of restoring worn away portions of open hearth furnace banks, to normal usable condition which consists in placing discrete refractory repair material in the cavities in the bank, covering said material with a thin layer of slag directly after a heat, and fusing the slag, permitting it to trickle into said material, whereby to bond said material together, adding additional refractory repair material to fill the cavities and covering the same with slag, and fusing the added slag whereby to bond the refractory repair materials together.

CHARLES A. HOGAN.

#### REFERENCES CITED

The following references are of record in the file of this patent:

#### UNITED STATES PATENTS

| Number    | Name     | Date          |
|-----------|----------|---------------|
| 714,565   | Dunford  | Nov. 25, 1902 |
| 1,670,098 | Brownlee | May 15, 1928  |
| 2,284,797 | Blau     | June 2, 1942  |

#### OTHER REFERENCES

Page 202 of "Modern Refractory Practice," 2nd edition, copyright 1937 and distributed by the Harbison-Walker Refractories Company, 30 Pittsburgh, Pa. (Copy in Div. 28.)

"The Making, Shaping and Treating of Steel," by Camp and Francis, pages 396, 397, 5th edition, 2nd impression, published by Carnegie-Illinois Steel Corporation, subsidiary in Pittsburgh, Pa., 35 and Chicago, Ill. (Copy in Div. 28.)